

# UNITED STATES PATENT OFFICE.

GEORGE FUNES DIEZ, OF NEW YORK, N. Y.

## PROCESS OF PRODUCING STEEL DIES.

No. 857,926.

Specification of Letters Patent.

Patented June 25, 1907.

Application filed February 5, 1907. Serial No. 365,954.

*To all whom it may concern:*

Be it known that I, GEORGE FUNES DIEZ, a citizen of the United States, residing at New York, in the county of New York and State of New York, have invented a new and useful Process of Producing Steel Dies, of which the following is a specification.

This invention has reference to improvements in the process of producing steel dies directly from the object to be reproduced without the necessity of engraving the die.

The invention consists essentially in depositing iron electrolytically directly upon the surface to be reproduced and then in so treating the iron matrix thus formed as to convert it into a grade of steel best suited for producing positive impressions in the material chosen for the copies of the original.

The improved process is particularly applicable for the reproduction of the finest type of engraving where faithfulness of the copy is important, since I am enabled to produce directly upon the body to be copied a film of exceeding fineness, so fine and homogeneous in texture as to produce a deposit which from beginning to end is white like tin and at the same time so free from corrugations, roughness or crystalline structure as to have the softness of silk to the touch. In this respect the deposited iron is far superior to copper for the copying of all kinds of metals, coins, etc., and it has the further advantage that the iron copy can be converted into steel of any degree of hardness so that it may be used directly for making positive copies of the original.

In carrying out my improved process, I first prepare a bath by taking 1000 cubic centimeters of a saturated aqueous solution 40 of iron sulfate and 125 cubic centimeters of a saturated aqueous solution of sodium bicarbonate. To prepare this bath, which is to constitute the electrolyte, I first mix with the 1000 cubic centimeters of the saturated solution of iron sulfate but one-half of the saturated solution of sodium bicarbonate, or 62½ cubic centimeters of the latter. The mixture is stirred with a wooden rod and allowed to stand for twelve hours, after which it is filtered and the remainder of the saturated solution of sodium bicarbonate is added and the bath is then permitted to stand for twenty-four hours. The electrolyte is placed in a tank or vat of glass, porcelain, varnished wood or other suitable material, and the ob-

jects to be plated or copied are hung in the vat and are connected up to a suitable source of electric current so that they constitute the cathode. The anode is composed of an iron plate. For the best results the current should range between 0.7 and 1.5 volts, while the density of the bath must be from 18 to 20 degrees Baumé, and the temperature should be about 21 degrees centigrade if it is desired to deposit the metal rapidly, but a temperature as low as 16 degrees centigrade is quite practicable.

The molds constituting the cathode are hung by fine copper wire from suitable supports in the usual manner and are located from 10 to 25 centimeters from the anode. The deposit of iron begins at once simultaneously over all the surface of the mold and the color is a velvety, metallic white. It will be understood, of course, that any material which it is desired to copy which in itself is not electro-conducting will be treated so as to form a conducting film over the surface to be copied. The time during which the molds should be kept in the bath will depend upon the desired thickness of metal to be obtained. Under normal conditions a matrix thick enough for type or for seals to stamp on leather or paper can be obtained in from three to four days, depending on the dimensions, while a matrix to be attached to a block of steel and used as a die to stamp on metals will require from ten to fifteen days.

In order to separate the deposited metal from the original or master, it is taken from the bath and washed with distilled water, after which, if the mold be metallic, the mold and matrix may be heated and may then be separated by inserting a thin blade between them and carefully prying them apart. If the original be of rubber, a slight heating will be sufficient, while when waxy compositions are used, an immersion in boiling water is all that is necessary.

The electrolytically deposited iron matrix is too soft for use and must therefore be converted into steel of the requisite hardness. For this purpose I take charcoal powder 8 parts, steel filings 1½ parts, potassium ferrocyanide ½ part. To this mixture I add a sufficient quantity of oil to form a paste. The several ingredients are all ground together in a mortar and the oil is added in small quantities from time to time until the desired paste is formed. The crucible is half filled

with the paste and the matrix is first wet with oil and then covered with powdered charcoal until a coating is formed thereon and is then placed in the crucible with the 5 matrix face down, after which the crucible is filled with the paste and pressed down and covered with plaster. The crucible is then placed in an oven and maintained at a red heat from eight to ten hours, when the plate 10 will be found to be converted into the finest steel, after which it may be tempered and is ready for use for stamping metals, and will stand the pressure of the most powerful presses.

15 All the details of the original from which the matrix has been produced will be found so perfectly reproduced that retouching is not required. The bath will work perfectly and regularly for many months and it is only 20 necessary to clean the anode from time to time since it may contain impurities which will form a black coating and must be cleaned off. It is also necessary from time to time to add some of the saturated solution of 25 sodium bicarbonate so as to make up losses due to evaporation and to maintain the level of the bath. The sodium bicarbonate serves to remove the oxid from the body of the liquid, which oxid rises to the surface and 30 there forms a film consistent enough to serve as a cover to the bath, thus keeping it free from such impurities as might reach it from the air.

I claim:—

1. The method of depositing iron upon a 35 conducting surface consisting in subjecting the surface to be copied to the action of an electric current in an electrolyte containing iron sulfate and sodium bicarbonate.

2. The method of depositing iron upon a 40 conducting surface consisting in subjecting the surface to be copied to the action of an electric current in an electrolyte composed of iron sulfate and sodium bicarbonate, and maintaining the strength of the bath 45 constant by the presence of an iron anode.

3. The method of producing iron matrices of conducting surfaces consisting in depositing the iron electrolytically upon said surfaces in an electrolyte consisting of a saturated solution of iron sulfate and a saturated 50 solution of sodium bicarbonate.

4. The method of producing iron matrices of conducting surfaces consisting in depositing the iron electrolytically upon said surfaces in an electrolyte consisting of about 55 eight parts of a saturated solution of iron sulfate and about one part of a saturated solution of sodium bicarbonate.

In testimony that I claim the foregoing as 60 my own, I have hereto affixed my signature in the presence of two witnesses.

GEORGE FUNES DIEZ.

Witnesses:

F. A. RANELLA,  
MANUEL RODRIGUEZ.